

## 1

2,737,493

## LITHIUM SOAP GREASE WITH PHOSPHATE ESTER VEHICLE

Richard A. Butcosk, East Hempstead, N. Y., assignor to Socony Mobil Oil Company, Inc., a corporation of New York

No Drawing. Application December 26, 1952,  
Serial No. 328,133

13 Claims. (Cl. 252—36)

This invention has to do with lubricating grease compositions suitable for use over a wide range of operating temperatures. More specifically, the present invention is concerned with lithium base greases of excellent lubricating character and stable when used at temperatures varying from about -70° F. to about 300° F. and higher.

In recent years, a demand has been created for greases of outstanding lubricating character which retain their grease structure during use over a wide range of operating temperatures. Typical of such a demand is that created by the aircraft industry. For efficient aircraft operation, greases should have low temperature torque properties such that they will flow properly at temperatures as low as about -70° F. In addition, the greases should be of low volatility and retain their grease structure at temperatures at least as high as 300° F. Failure to retain grease structure results in high consumption of grease and frequent servicing. Other desirable features of such greases are: homogeneity and smooth, uncrossed consistency; water resistance; resistance to oxidation; resistance to oil separation; and resistance to shear or breakdown upon working or milling.

The demand for greases of the foregoing specification has not been satisfied to date, except by resort to expensive operating procedures. It has been found, for example, that lithium base greases containing synthetic vehicles comprising esters of dibasic acids, such as di-(2-ethyl-hexyl) sebacate and di-(iso octyl) adipate, are suitable for low temperature operations; and, in fact, such greases are used in aircraft, as reflected in Military Specification MIL-G-3278. The latter greases have the desired homogeneous nature and smooth consistency, and have satisfactory water resistance. Yet, these lithium base greases have a weakness in that their ester vehicles have excess volatility at temperatures of 300° F. and higher. Such a loss is too great for long service life of the greases in anti-friction bearings. Another shortcoming of such greases is their lack of extreme pressure (E. P.) properties, necessitating incorporation of an additive material imparting E. P. characteristics. One approach taken to effect improvement of lithium base greases involves a special film-cooling technique to obtain satisfactory grease structure. As will be evident to those skilled in the art, film-cooling is a slow and expensive procedure requiring special equipment. Another approach taken to effect such improvement involves the use of a lithium soap of 12-hydroxy stearic acid and quick cooling. Still another approach involves the use of a very high soap content grease. Still another means adopted to improve grease structure is the use of a mixed soap, namely the use of a calcium soap in admixture with the lithium soap. However, lithium-calcium base greases are deficient in mechanical stability and have lower melting points, thus requiring their use at lower operating temperatures (e. g., below 250° F.).

It is an object of this invention, therefore, to provide a grease effective over a wide temperature range, particularly from about -70° F. to about 300° F. A fur-

## 2

ther object is to provide a grease which retains its original character over a wide range of operating conditions. Another object is to provide a grease with extreme pressure properties furnished by the oil vehicle rather than by an E. P. additive. Still another object is to provide a grease characterized by a relatively low degree of volatility. Another object is to provide a grease of desired character which can be manufactured by conventional grease procedures in conventional grease-making equipment. Other objects of the invention will be apparent from the following description.

It has now been discovered that lithium base greases containing vehicles comprising alkyl, aryl phosphate esters, and containing small amounts of particular lithium or aluminum salts, in certain proportions, make possible realization of the foregoing objects.

The vehicles or synthetic oils of the greases contemplated herein are confined to alkyl, aryl phosphate esters, represented by the following general formula:



wherein R is alkyl, R<sub>1</sub> is aryl and R<sub>2</sub> is either alkyl or aryl, typical of which groups are: (1) alkyl such as methyl, ethyl, propyl, butyl, amyl, 2-ethyl hexyl, iso octyl, etc. (2) aryl such as phenyl, and its alkylated derivatives such as cresyl, amyl phenyl and the like. Representative of such esters are: dibutyl, mono-phenyl phosphate; di-(2-ethyl-hexyl), monophenyl phosphate; and mono-iso octyl, diphenyl phosphate. Particularly advantageous of such esters is dibutyl, mono phenyl phosphate.

In general, the synthetic vehicles described above and contemplated for use in the greases of this invention have a viscosity from about 40 seconds to about 150 seconds, S. U. V. at 100° F. Particularly desirable are those having a viscosity of the order of 50 to 60 seconds, S. U. V., at 100° F. The vehicles also have low pour points and low evaporation rates at elevated temperatures.

Physical characteristics of several typical phosphate esters are presented below in Table I.

Table I

|                        | Di (2 Ethyl Hexyl),<br>Mono Phenyl<br>Phosphate | Di Butyl,<br>Mono<br>Phenyl<br>Phosphate | Iso Octyl,<br>Diphenyl<br>Phosphate |
|------------------------|-------------------------------------------------|------------------------------------------|-------------------------------------|
| 50 Flash, C. O. C. °F. | 385                                             | 370                                      | 455                                 |
| Fire, C. O. C. °F.     | 460                                             | 395                                      | 430                                 |
| Visc. @ 100° F., SUS   | 54                                              | 52                                       | 61                                  |
| Visc. @ 210° F., SUS   | 34                                              | 36                                       | 35                                  |
| Viscosity Index        | 80                                              | 205                                      | 73                                  |
| Pour, °F.              | Below -60                                       | Below -70                                | Below -60                           |
| Specific Gravity       | 0.9916                                          | 1.0663                                   | 1.097                               |

The lithium fatty acid soap constituting one of the soap or gelling components of the greases of this invention, is prepared with a fat or fatty material containing from about twelve to about twenty-two carbon atoms per molecule. Representative of such materials are vegetable, animal and fish fatty oils, and hydrogenated materials thereof. Stearin, stearic acid, cottonseed oil acids, oleic acid, palmitic acid, myristic acid, 12-hydroxy stearic acid, hydrogenated fish oils such as "Hydrogenated Fish Oil, Iodine No. 77" and "Hydrofol" are typical. Preferred soaps, however, are lithium stearate and the lithium soap of 12-hydroxy stearic acid. Methods of preparation of lithium soaps are well known in the art and, for this reason, detailed discussion of the same is omitted.

The lithium and aluminum salts contemplated herein as modifying agents are salts of aliphatic monocarboxylic

acids having from about six to about ten carbon atoms per molecule. Typical of such salts are lithium and aluminum salts of: hexanoic, heptanoic, octoic such as caprylic and 2-ethyl hexanoic, pelargonic and decanoic. Particularly preferred herein are lithium and aluminum octoates.

In connection with the above-mentioned modifying agents, it has been found that satisfactory grease gels could not be formed from the phosphate ester vehicles and lithium soaps described above when the modifying salts were absent. It has also been found that conventional metal soap types, such as calcium and magnesium stearates do not form gels with the phosphate esters with or without the modifying salts. It was further found that when certain proportions of the lithium and/or aluminum salt modifying agents were used with the phosphate ester vehicles and lithium soaps, excellent grease gels could be formed. The lithium and/or aluminum salts are used in amounts of the order of 0.2 per cent to about ten per cent by weight of the grease. Generally, however, particularly advantageous behavior is realized with from about one to about three per cent of the modifying agent, with balanced proportions of the phosphate ester vehicle and lithium soap. The latter comprises from about four to about thirty per cent of the grease, and the vehicle from about sixty to about ninety-four per cent of the grease. For convenience, these balanced proportions are shown below in tabulated form:

|                                                            | General | Preferred |
|------------------------------------------------------------|---------|-----------|
| Lithium Soaps.....                                         | 4-30    | 8-15      |
| Lithium and/or Aluminum Salt.....                          | 0.2-10  | 1-3       |
| Phosphate Ester Vehicle—Balance to 100 per cent, e. g..... | 60-94   | 82-91     |

It is to be understood that the greases of this invention can also contain other characterizing ingredients. For

example, they can contain lubricity improving agents such as free fat, free fatty acids, esters of alkyl and/or aryl esters, sulfurized fats, lead soaps, etc. These characterizing materials do not detract from the lubricating

5 value of the greases contemplated herein nor do they detract from the beneficial properties imparted by the lithium soap and the lithium and/or aluminum salt; rather, these characterizing materials serve to impart their customary properties to the grease. In general, the characterizing material or materials are present, in total, in amounts up to about five per cent by weight of the grease.

By way of illustration, the greases of this invention can be formed in the following manner. A preformed 15 lithium soap and a preformed lithium and/or aluminum salt are mixed well at room temperature, about 70-80° F. with a phosphate ester vehicle. The resultant mixture is heated to a temperature from about 90° F. to about 500° F., preferably about 420° F., with constant 20 stirring, during a period of thirty minutes to about two hours, depending upon the quantities of materials used. After the time period indicated above, the resulting liquid product is cooled to room temperature, generally requiring a period of about one to ten hours. The cooled 25 grease product is milled to a buttery product in a suitable milling apparatus, such as Cornell homogenizer. When any additives are incorporated in the greases it is advisable to add them just prior to cooling the products.

The greases of this invention are illustrated by several 30 examples—1 through 5—tabulated in Table II below. Provided also in Table II are comparable examples in which lithium base greases and other metal base greases, other than those contemplated herein are illustrated. Each of the greases shown in Table II was prepared according to the procedure described above, unless otherwise indicated. Consistency of the greases was determined in accordance with ASTM Method D 217-48 "Cone Penetration of Lubricating Grease."

Table II

| Grease No.....                                        | 1              | 2            | 3              | 4               | 5            | 6            | 7                |
|-------------------------------------------------------|----------------|--------------|----------------|-----------------|--------------|--------------|------------------|
| Ingredients:                                          |                |              |                |                 |              |              |                  |
| Lithium Stearate..... percent by weight.....          | 20.00.....     |              |                | 4.00.....       | 20.00.....   |              |                  |
| Lithium Palmitate..... do.....                        | 20.00.....     |              |                |                 |              |              |                  |
| Lithium 12 Hydroxystearate..... do.....               | 15.00.....     |              |                |                 |              |              |                  |
| Aluminum Octoate..... do.....                         | 2.00.....      | 2.00.....    | 2.00.....      |                 |              |              |                  |
| Lithium Octoate..... do.....                          |                |              |                |                 |              |              |                  |
| Lithium Laurate..... do.....                          |                |              |                |                 | 2.00.....    | 10.00.....   | 20.00.....       |
| Dibutyl, Monophenyl Phosphate..... do.....            | 78.00.....     | 78.00.....   | 83.00.....     | 92.00.....      | 78.00.....   | 90.00.....   | 80.00.....       |
| Iso Octyl, Diphenyl Phosphate..... do.....            | 268.....       | 265.....     | 260.....       | 300.....        | 350.....     | 400.....     | 390.....         |
| Consistency.....                                      | 268.....       | 265.....     | 260.....       | 300.....        | 350.....     | 400.....     | 390.....         |
| Structure.....                                        | Smooth.....    | Smooth.....  | Smooth.....    | Sl. Grainy..... | Grainy.....  | Grainy.....  | Grainy.....      |
| Appearance.....                                       | Buttery.....   | Buttery..... | Buttery.....   | Buttery.....    | Buttery..... | Fibrous..... | Buttery.....     |
| Grease No.....                                        | 8              | 9            | 10             | 11              | 12           | 13           | 14               |
| Ingredients:                                          |                |              |                |                 |              |              |                  |
| Lithium Stearate..... percent by weight.....          | 15.00.....     | 15.00.....   | 20.00.....     |                 | 20.00.....   |              | 20.00.....       |
| Lithium Palmitate..... do.....                        |                |              |                | 20.00.....      |              |              | 20.00.....       |
| Lithium 12 Hydroxystearate..... do.....               |                |              |                |                 | 15.00.....   |              |                  |
| Calcium Stearate..... do.....                         |                | 3.00.....    |                |                 |              |              |                  |
| Aluminum Stearate..... do.....                        |                |              |                |                 |              | 2.00.....    |                  |
| Aluminum Caprylate..... do.....                       |                |              |                |                 |              |              | 2.00.....        |
| Lithium Caprylate..... do.....                        |                |              |                |                 |              |              | 2.00.....        |
| Dibutyl, Monophenyl Phosphate..... do.....            |                |              |                |                 |              |              |                  |
| Iso Octyl, Diphenyl Phosphate..... do.....            |                |              |                |                 | 80.00.....   | 85.00.....   | 78.00.....       |
| D-1-2-Ethyl-Hexyl), Monophenyl Phosphate..... do..... | 85.00.....     | 82.00.....   | 80.00.....     | 80.00.....      |              |              | 78.00.....       |
| Consistency.....                                      | Semifluid..... | Fluid.....   | Semifluid..... | Semifluid.....  |              |              | 78.00.....       |
| Appearance.....                                       | Grainy.....    | Grainy.....  | Grainy.....    | Grainy.....     | Grainy.....  | Grainy.....  | 400. Grainy..... |
| Grease No.....                                        | 15             | 16           |                |                 |              |              |                  |

Table II.—Continued

| Grease No.                                              | 17     | 18        | 19        | 20     | 21        | 22        | 23     | 24     | 25 <sup>1</sup> |
|---------------------------------------------------------|--------|-----------|-----------|--------|-----------|-----------|--------|--------|-----------------|
| <b>Ingredients:</b>                                     |        |           |           |        |           |           |        |        |                 |
| Magnesium Stearate<br>percent by weight                 | 20.00  |           |           |        | 15.00     |           |        |        |                 |
| Calcium Stearate<br>do                                  |        | 15.00     |           | 15.00  |           |           |        |        |                 |
| Aluminum Stearate<br>do                                 |        |           | 15.00     | 2.00   | 2.00      | 10.00     |        |        |                 |
| Aluminum Octoate<br>do                                  |        |           |           |        |           |           | 20.00  |        |                 |
| Calcium Laurate<br>do                                   |        |           |           |        |           |           |        |        |                 |
| Lithium Alpha Hydroxy<br>Decanoate<br>percent by weight |        |           |           |        |           |           |        | 20.00  | 20.00           |
| Lithium Stearate<br>do                                  |        |           |           |        |           |           |        |        | 20.00           |
| Dibutyl, Monophenyl Phosphate<br>percent by weight      |        |           |           |        |           | 90.00     |        |        |                 |
| Iso Octyl, Diphenyl Phosphate<br>percent by weight      | 80.00  | 85.00     | 85.00     | 83.00  | 83.00     |           | 80.00  | 80.00  | 80.00           |
| Consistency                                             | Fluid  | Semifluid | Semifluid | Fluid  | Semifluid | Semifluid | 420    | 420    | 360             |
| Appearance                                              | Grainy | Grainy    | Grainy    | Grainy | Grainy    | Grainy    | Grainy | Grainy | Sl. Grainy.     |

<sup>1</sup> Experiment 25 was prepared like previous experiments but the mixture was agitated during cooling to 90° F. over a period of 45 minutes.

In reviewing the results set forth in Table II, it will be noted that greases 1 through 5 represent compositions of the present invention. Greases 1 through 4 are smooth textured. The greases of this invention are suitable for lubrication of ball and roller bearings at low and elevated temperatures. In addition, they are characterized by low volatility at high temperatures and are further characterized by excellent film strength properties.

As a further note in connection with greases 1 through 5, each of such greases in addition to being pan cooled, was shock cooled. Each grease was poured, while hot, onto a cool surface and then worked with a spatula. The resultant greases were firm, just as they were when obtained by the pan cooling technique. In contrast, greases 8 through 24 were unsatisfactory when shock cooled.

Greases 6 and 7 are unsatisfactory because they are grainy and approach a semi-fluid consistency.

Greases 8 through 24 are semi-fluid and grainy in nature, and are unsatisfactory. Grease 25 is slightly grainy and soft in consistency; it was kettle cooled, or agitated during cooling, from 420° F. to 90° F. over a period of two hours.

The greases of this invention are suitable for a wide range of industrial applications. They are, as indicated above, particularly well suited for use in aircraft, such as applied to wheel bearings, ball bearing motors, actuators.

I claim:

1. A lubricating grease comprising: at least 60 percent by weight of a dialkyl monoaryl phosphate ester vehicle, a lithium fatty acid soap (I) in an amount from about four to about thirty per cent by weight of the grease, and a metal salt (II) of a monocarboxylic aliphatic acid having from about six to about ten carbon atoms per molecule in an amount from about 0.2 to about ten per cent by weight of the grease, the metal of said metal salt (II) being selected from the group consisting of lithium and aluminum.

2. A grease defined by claim 1 wherein the vehicle is an ester represented by the general formula



wherein R and R<sub>1</sub> are alkyl groups, and R<sub>2</sub> is an aryl group.

3. A grease defined by claim 1 wherein the vehicle is dibutyl, monophenyl phosphate.

4. A grease defined by claim 1 wherein the lithium soap is lithium stearate.

5. A grease defined by claim 1 wherein the metal salt is lithium octoate.

6. A grease defined by claim 1 wherein the metal salt is aluminum octoate.

7. A lubricating grease comprising:

- Per cent by weight
- 20 A dialkyl monoaryl phosphate ester vehicle 82-91
- 20 A metal salt (II) of a monocarboxylic aliphatic acid having from about six to about ten carbon atoms per molecule, the metal of said salt (II) being selected from the group consisting of lithium and aluminum 1-3
- 25 A lithium fatty acid soap (I) 8-15
- 30 8. A lubricating grease comprising about seventy-eight per cent by weight of dibutyl, monophenyl phosphate, about twenty per cent by weight of lithium stearate and about two per cent by weight of aluminum octoate.
- 35 9. A lubricating grease comprising about seventy-eight per cent by weight of dibutyl, monophenyl phosphate, about twenty per cent by weight of lithium palmitate and about two per cent by weight of aluminum octoate.
- 35 10. A lubricating grease comprising about eighty-three per cent by weight of dibutyl, monophenyl phosphate, about fifteen per cent by weight of lithium 12-hydroxy stearate and about two per cent by weight of aluminum octoate.
- 40 11. A lubricating grease comprising about ninety-two per cent by weight of dibutyl, monophenyl phosphate, about four per cent by weight of lithium stearate and about four per cent by weight of aluminum octoate.
- 45 12. The method for preparing a lithium soap lubricating grease, which comprises mixing a lithium fatty acid soap (I) in an amount from about four to about thirty per cent by weight of the total charge, with a metal salt (II) in an amount from about 0.2 to about ten per cent by weight of the total charge, and with the balance a vehicle consisting of a dialkyl monoaryl phosphate ester, said metal salt (II) being a salt of a monocarboxylic aliphatic acid having from about six to about ten carbon atoms per molecule and the metal thereof being selected from the group consisting of lithium and aluminum; heating the resultant mixture to a temperature from about 90° F. to about 500° F., while agitating said mixture, for a period of time from about 1/2 hour to about four hours; cooling and milling the grease product.
- 55 13. The method as defined by claim 12 wherein the resultant mixture is heated to a temperature of about 420° F.

References Cited in the file of this patent

UNITED STATES PATENTS

- 2,203,102 Powers June 4, 1940
- 2,237,336 Caprio Apr. 8, 1941
- 2,376,312 Morgan May 15, 1945
- 2,455,892 Fraser Dec. 7, 1948
- 2,487,080 Swenson Nov. 8, 1949
- 2,495,651 Butcosk Jan. 24, 1950
- 70 2,585,321 Butcosk Feb. 12, 1952
- 2,614,076 Moore et al. Oct. 14, 1952
- 2,614,077 Moore et al. Oct. 14, 1952
- 2,628,195 Allison et al. Feb. 10, 1953
- 2,628,202 Allison et al. Feb. 10, 1953
- 75 2,651,616 Matthews et al. Sept. 8, 1953